

## UNITED STATES PATENT OFFICE

BENNO STRAUSS, OF ESSEN-BREDENEY, GERMANY, ASSIGNOR TO FRIED. KRUPP AKTIENGESELLSCHAFT, OF ESSEN-ON-THE-RUHR, GERMANY

## STEEL ALLOY INSENSIBLE TO HOT GASES AND VAPORS

No Drawing. Application filed April 5, 1929, Serial No. 352,912, and in Germany September 21, 1928.

In the conversion of oil residues to gasoline the steel vessels used to perform the reactions are exposed to the action of the products of decomposition of the oil at elevated temperatures (about 550 degrees C.) and under high pressures (up to 70 atm.). As practice has shown, these vessels very soon become short. The invention has for its object to afford a steel which is rendered insensitive to the action of hot gases and vapors to the process described in my co-pending patent application Serial Number 149,282, filed November 18th, 1926, which new steel possesses the advantageous property of not becoming short even when exposed to the action of the products of decompositon of the oils at high temperatures (about 550 degrees C.) and under high pressures (about up to 70 atm.). This object is obtained according to the invention by having the steel alloy used for the manufacture of the vessels contain about 0.1 to 0.2 per cent of carbon, 5 to 12 per cent of chromium, 0.2 to 0.5 per cent of vanadium, with or without  $\frac{1}{2}$  to 2 per cent of nickel.

The following steel alloy, e. g. has been proved to be particularly well suited for the manufacture of the indicated vessels, viz. an alloy containing about 0.15 per cent of carbon, 6 per cent of chromium, 0.3 per cent of vanadium, 2 per cent of nickel.

Vessels made of the above steel alloys do not become short even when exposed to high temperatures and pressures in the conversion of oil residues to gasoline, because these steel alloys in a particularly high degree are free of grain boundaries if treated by the process described in my co-pending patent application Serial Number 149,282, filed November 18th, 1926. This process consists in heating the alloy above the critical point  $Ac_3$  quickly cooling it, and then re-heating to about 600 to 650° C.

I claim:

1. As a new article of manufacture vessels adapted to be used in the conversion of oil residues to gasoline and consisting of an alloy that has been heated above the critical point  $Ac_3$ , quickly cooled, and re-heated to about 600° to 650° C. said alloy

being composed of 0.1 to 0.2 per cent of carbon, 5 to 12 per cent of chromium, 0.2 to 0.5 per cent of vanadium, the remainder steel.

2. As a new article of manufacture vessels 55 adapted to be used in the conversion of oil residues to gasoline and consisting of an alloy that has been heated above the critical point  $Ac_3$ , quickly cooled, and re-heated to about 600° to 650° C., said alloy being composed of 0.1 to 0.2 per cent of carbon, 5 to 12 per cent of chromium, 0.2 to 0.5 per cent of vanadium,  $\frac{1}{2}$  to 2 per cent of nickel, the remainder steel.

3. As a new article of manufacture vessels 65 adapted to be used in the conversion of oil residues to gasoline and consisting of an alloy that has been heated above the critical point  $Ac_3$ , quickly cooled, and re-heated to about 600° to 650° C., said alloy being composed of 0.15 per cent of carbon, 6 per cent of chromium, 2 per cent of nickel, 0.3 per cent of vanadium, the remainder steel.

The foregoing specification signed at Cologne, Germany, this 20th day of March, 70 1929.

BENNO STRAUSS.

80

85

90

95

100